



US009364890B2

(12) **United States Patent**  
**Foltz, IV et al.**

(10) **Patent No.:** **US 9,364,890 B2**  
(b4) **Date of Patent:** **Jun. 14, 2016**

(54) **ENHANCED TECHNIQUES FOR CENTRIFUGAL CASTING OF MOLTEN MATERIALS**

(71) Applicant: **ATI PROPERTIES, INC.**, Albany, OR (US)

(72) Inventors: **John W. Foltz, IV**, Albany, OR (US); **Raul A. Martinez-Ayers**, Albany, OR (US); **Aaron L. Fosdick**, Albany, OR (US)

(73) Assignee: **ATI PROPERTIES, INC.**, Albany, OR (US)

(\*) Notice: Subject to any disclaimer, the term of this patent is extended or adjusted under 35 U.S.C. 154(b) by 161 days.

(21) Appl. No.: **14/169,665**

(22) Filed: **Jan. 31, 2014**

(65) **Prior Publication Data**

US 2015/0352633 A1 Dec. 10, 2015

**Related U.S. Application Data**

(63) Continuation-in-part of application No. 13/792,929, filed on Mar. 11, 2013.

(51) **Int. Cl.**

**B22C 9/08** (2006.01)

**B22D 13/06** (2006.01)

**B22D 13/10** (2006.01)

**B22D 27/04** (2006.01)

(52) **U.S. Cl.**

CPC . **B22C 9/08** (2013.01); **B22D 13/06** (2013.01);

**B22D 13/066** (2013.01); **B22D 13/101**

(2013.01); **B22D 13/107** (2013.01); **B22D**

**27/045** (2013.01)

(58) **Field of Classification Search**

CPC ..... B22D 13/00; B22D 13/066; B22D 13/06; B22D 13/107; B22D 13/10

See application file for complete search history.

(56) **References Cited**

**U.S. PATENT DOCUMENTS**

2,107,513 A \* 2/1938 Swoger ..... B22D 13/04 164/291

4,519,971 A 5/1985 Schaer

5,119,865 A 6/1992 Mae et al.

5,311,655 A 5/1994 Jager et al.

(Continued)

**FOREIGN PATENT DOCUMENTS**

DE 19639514 C1 12/1997  
EP 0686443 A1 12/1995

(Continued)

**OTHER PUBLICATIONS**

Achtermann et al., "Production of  $\gamma$ -TiAl based feed stock materials for subsequent investment casting and forging operations", Sep. 15, 2011, Gfe, 24 pages.

(Continued)

*Primary Examiner* — Kevin P Kerns

*Assistant Examiner* — Steven Ha

(74) *Attorney, Agent, or Firm* — K&L Gates LLP

**ABSTRACT**

Various enhanced features are provided for centrifugal casting apparatuses, rotatable assemblies, and molds for casting products from molten material. These enhanced features include, among others, tapered gate portions positioned adjacent to the cavities of a mold, extended and shared gating systems, and detachable mold structures for modifying the thermodynamic characteristics and behavior of molds during casting operations.

**20 Claims, 23 Drawing Sheets**



(56)

**References Cited**

U.S. PATENT DOCUMENTS

6,443,212 B1 9/2002 Choudhury et al.  
6,499,529 B1 12/2002 Farkas  
6,705,385 B2 3/2004 Ray et al.  
6,776,214 B2 8/2004 Ray et al.  
6,935,406 B2 8/2005 Flemings et al.  
8,136,572 B2 3/2012 Renkel  
8,347,485 B2 1/2013 Biederman et al.  
2003/0042001 A1 \* 3/2003 Ray ..... B22C 3/00  
164/529  
2012/0207611 A1 8/2012 Luckow et al.  
2014/0251570 A1 9/2014 Foltz et al.

## FOREIGN PATENT DOCUMENTS

JP 03189057 A \* 8/1991  
JP 8-206807 A 8/1996  
JP 8-238555 A 9/1996

## OTHER PUBLICATIONS

Casting (metalworking), Wikipedia, [http://en.m.wikipedia.org/wiki/Casting\\_\(metalworking\)](http://en.m.wikipedia.org/wiki/Casting_(metalworking)), 23 pages.

\* cited by examiner



FIG. 1  
PRIOR ART



FIG. 2



FIG. 3



FIG. 4



FIG. 5



6  
FIG





FIG. 8



FIG. 9



FIG. 10



FIG. 11



FIG. 12



FIG. 13



FIG. 14



FIG. 15



FIG. 16





FIG. 17



FIG. 18



FIG. 19



FIG. 20



FIG. 21

FIG. 22



## 1

**ENHANCED TECHNIQUES FOR  
CENTRIFUGAL CASTING OF MOLTEN  
MATERIALS**

**CROSS-REFERENCE TO RELATED  
APPLICATIONS**

The present application is a continuation-in-part of co-pending U.S. patent application Ser. No. 13/792,929, filed on Mar. 11, 2013, the disclosure of which is hereby incorporated by reference in its entirety.

**BACKGROUND OF THE TECHNOLOGY**

1. Field of the Technology

The present disclosure generally relates to equipment and techniques for centrifugal casting. The present disclosure more specifically relates to equipment and techniques for centrifugal casting of metallic materials.

2. Description of the Background of the Technology

Metallic casting generally includes supplying a volume of molten metallic material to a static or rotating mold and allowing the material to cool to produce a casting shaped by the mold. Castings may be cast in near net form or may be further modified in subsequent forging or machining applications to produce final components. Metallic materials shrink during phase transition from liquid to solid, which may result in castings comprising uncontrolled shrinkage porosity, especially in difficult to cast metallic materials such as, for example, titanium aluminide (TiAl) based alloys and other TiAl materials. Shrinkage porosity is inherent to the fundamental solidification mechanics and may negatively impact microstructure as well as casting yield. In general, minimized internalized porosity may be addressed by processing techniques such as hot isostatic pressing (HIP). However, uncontrolled internal porosity may result in surface distortions affecting surface quality of the casting and increase production costs. Uncontrolled internal porosity may also be exposed when castings are sectioned or separated from casting components. When porosity is surface connected, current processing techniques may be unsuitable for many casting applications. For example, surface treatment techniques designed to fill or enclose porosity may fail to maintain the continuity of the casting, which may detrimentally affect mechanical properties of the cast material. Material removal techniques such as machining to remove external porosity may also reduce casting yield and expose additional porosity.

Conventional casting techniques for casting various metallic materials, such as titanium aluminide based alloys, are incapable of controlling porosity such that the porosity is internalized away from both the surface of a casting and regions of the casting that may be subsequently sectioned. For example, others have described preparation of titanium aluminide sections using a series of static casting and vacuum arc remelting techniques. These static casting techniques, however, create significant porosity, which cannot be removed using HIP. Others have also described centrifugal casting techniques for preparation of titanium aluminide castings that require supplying molten material to the centrifuge before the centrifuge reaches rotational speed. Cooling rate and solidification, however, are difficult to control, as is evident by the requirement of a separate heating method and mold for each cast piece. Although various other centrifugal casting techniques have been reported, none are able to adequately control shrinkage porosity.

Given the drawbacks associated with conventional casting techniques for casting metallic materials, including centrifu-

## 2

gal casting techniques, it would be advantageous to develop improved techniques for casting metallic materials.

**SUMMARY OF THE TECHNOLOGY**

5

According to one aspect of the present disclosure, an embodiment of a mold is structured for operative association with a rotatable assembly of a centrifugal casting apparatus. The mold may include at least one cavity having an entry port structured to receive molten material in a general direction of centrifugal force generated by rotation of the rotatable assembly. Also, a gate within the mold may be in communication with the entry port of the cavity, wherein the gate includes at least one tapered portion positioned adjacent to the entry port of the cavity.

10

According to one aspect of the present disclosure, an embodiment of a mold is structured for operative association with a rotatable assembly of a centrifugal casting apparatus. The mold may include at least one cavity having an entry port structured to receive molten material in a general direction of centrifugal force generated by rotation of the rotatable assembly. Also, the mold may include an extended gate in communication with the entry port of the cavity and the cavity can be structured for producing a cast component capable of subdivision into multiple sub-components having a predefined aspect ratio.

15

According to one aspect of the present disclosure, an embodiment of a mold is structured for operative association with a rotatable assembly of a centrifugal casting apparatus. The mold may include at least two cavities each having an entry port structured to receive molten material in a general direction of centrifugal force generated by rotation of the rotatable assembly. The cavities may share a common gate in communication with both entry ports of the cavities.

20

According to one aspect of the present disclosure, an embodiment of a mold is structured for operative association with a rotatable assembly of a centrifugal casting apparatus. The mold may include at least one cavity having an entry port structured to receive molten material in a general direction of centrifugal force generated by rotation of the rotatable assembly. Also, the mold may include a main body portion comprising a first material, and a back wall portion attachable or detachable to the main body portion, wherein the back wall portion comprises a second material. The first and second materials may be different material types.

25

According to one aspect of the present disclosure, an embodiment of a mold is structured for operative association with a rotatable assembly of a centrifugal casting apparatus. The mold may include at least one cavity having an entry port structured to receive molten material from a gate in a general direction of centrifugal force generated by rotation of the rotatable assembly. Also, a slot may be formed adjacent to the entry port of the cavity, wherein the slot is structured to removably receive therein a side wall of the gate.

30

**BRIEF DESCRIPTION OF THE DRAWINGS**

Features and advantages of the apparatus and methods described herein may be better understood by reference to the accompanying drawings in which:

FIG. 1 is a semi-schematic illustration of a rotating assembly of a conventional centrifugal casting assembly;

FIG. 2 is a simplified semi-schematic depiction of certain components of a rotating assembly of a centrifugal casting apparatus according to various non-limiting embodiments of the present disclosure;

FIG. 3 is a perspective view of certain components of a rotating assembly of a centrifugal casting apparatus according to various non-limiting embodiments of the present disclosure;

FIG. 4 is a partially exploded view shown in perspective of certain components of the rotating assembly illustrated in FIG. 3 according to one non-limiting embodiment of the present disclosure;

FIG. 5 is a partially exploded view shown in perspective of certain components of the rotating assembly illustrated in FIG. 3, illustrating a table, a wedge, and a containment ring in cross-section taken along line 5-5 and in the direction of the arrows in FIG. 3, according to one non-limiting embodiment of the present disclosure;

FIG. 6 is a perspective view of certain components of a rotating assembly of a centrifugal casting apparatus according to various non-limiting embodiments of the present disclosure;

FIG. 7 is a cross-section, taken along line 7-7 and in the direction of the arrows in FIG. 6, illustrating certain components of the rotating assembly illustrated in FIG. 6 according to one non-limiting embodiment of the present disclosure;

FIG. 8 is a front view of a mold according to one non-limiting embodiment of the present disclosure;

FIG. 9 is a perspective view of certain components of a rotating assembly of a centrifugal casting apparatus according to various non-limiting embodiments of the present disclosure;

FIG. 10 is a perspective view of a cross-section of a mold according to one non-limiting embodiment of the present disclosure;

FIG. 11 is a perspective view of a mold according to various non-limiting embodiments of the present disclosure;

FIG. 12 is a perspective view of a cross-section through the first cavity of the mold illustrated in FIG. 11 according to one non-limiting embodiment of the present disclosure;

FIG. 13 is a perspective view of a cross-section through the second cavity of the mold illustrated in FIG. 11 according to one non-limiting embodiment of the present disclosure;

FIG. 14 is a perspective view of a cross-section through the third cavity of the mold illustrated in FIG. 11 according to one non-limiting embodiment of the present disclosure;

FIG. 15 is a perspective view of a cross-section through the fourth cavity of the mold illustrated in FIG. 11 according to one non-limiting embodiment of the present disclosure;

FIG. 16 illustrates a perspective view of portion of a gate including a tapered portion structured according to various embodiments of the present disclosure;

FIG. 16A schematically illustrates a plan view of a gate including a tapered portion structured according to various embodiments of the present disclosure;

FIG. 17 includes a perspective view of a portion of a mold structured with an extended gate according to various embodiments of the present disclosure;

FIG. 18 includes a perspective view of a portion (part solid and part transparent for purposes of illustration) of a mold structured with an extended gate according to various embodiments of the present disclosure;

FIG. 19 includes a perspective view of a portion of a mold structured with a common gate according to various embodiments of the present disclosure;

FIG. 20 includes a perspective view of a centrifugal casting apparatus including a rotatable assembly structured according to various embodiments of the present disclosure;

FIG. 21 includes a top plan view of the mold of FIG. 20; and,

FIG. 22 includes a perspective view of a portion of a mold structured according to various embodiments of the present disclosure.

The reader will appreciate the foregoing details, as well as others, upon considering the following detailed description of certain non-limiting embodiments of apparatuses and methods according to the present disclosure. The reader also may comprehend certain of such additional details upon carrying out or using the apparatuses and methods described herein.

#### DETAILED DESCRIPTION OF CERTAIN NON-LIMITING EMBODIMENTS

Metallic materials may generally include one or more metal elements, and in some cases also include one or more non-metal elements. Shrinkage porosity is inherent to the fundamental solidification mechanics of many such metallic materials when cast, which may negatively impact mechanical properties of castings. Present static and centrifugal casting techniques for various metallic materials, e.g., titanium aluminide based alloys, are incapable of controlling porosity in both the surface of a casting and in regions where the casting may be subsequently sectioned.

In various non-limiting embodiments, the present disclosure describes centrifugal casting apparatuses comprising rotatable assemblies and components thereof structured to control shrinkage porosity. For example, centrifugal force may be used to feed molten material, such as molten metallic material, into casting pores, thereby minimizing molten material starvation in the solidifying material. Controlled shrinkage porosity may generally include controlling the amount and/or location of shrinkage porosity within a casting such that it may be removed with subsequent processing. For example, controlled shrinkage porosity may include shrinkage porosity that is internalized, e.g., non-surface connected and/or minimized. In some non-limiting embodiments, shrinkage porosity may be internalized away from particular regions of castings such that the castings may be sectioned and/or removed from casting components or material without exposing internalized porosity to the atmosphere.

According to certain non-limiting embodiments, the disclosed centrifugal casting apparatuses and methods may streamline subsequent processing of various castings and eliminate standard production routes such as those used in investment casting. In contrast to conventional centrifugal casting devices, which often require assembly of sixty or more mold components, certain non-limiting embodiments of the centrifugal casting apparatuses disclosed herein comprise rotatable assemblies that may be assembled from fewer than a typical number of major components, significantly reducing setup time. In various non-limiting embodiments, castings may be heat treated and/or processed by HIP, for example. According to certain non-limiting embodiments, castings produced by the disclosed centrifugal casting apparatuses and methods may be suitable for subsequent use in forging or machining applications to produce final components for jet engines, turbochargers, or various high temperature components, for example.

The apparatuses and methods according to the present disclosure may be used in casting metallic materials. As used herein, metallic materials may comprise metal and metal alloys. Metallic materials include, for example, TiAl materials, which comprise, for example, TiAl based alloys. TiAl based alloys may include one or more alloying elements in addition to titanium and aluminum. In certain non-limiting embodiments, the present apparatuses and methods may be used to cast TiAl materials comprising titanium and about

25.0 to 52.1 atomic percent aluminum or about 14 to 36 weight percent aluminum. The disclosed centrifugal casting apparatuses and methods may be used to produce castings of TiAl materials comprising other percentages of aluminum and other alloying elements, without limitation of the above. It is also to be appreciated that while various non-limiting embodiments and beneficial features may be described herein in terms of TiAl based alloys and other TiAl materials, the disclosed apparatuses and methods are not so limited. Those having skill in the art will recognize that the disclosed apparatuses and methods may find wide application beyond TiAl materials, such as, for example and without limitation, metallic materials that suffer from shrinkage porosity or have other properties or characteristics similar to TiAl materials. While certain non-limiting embodiments may provide significant advantages over conventional casting techniques when applied to TiAl materials, it is to be understood that the apparatuses and methods disclosed herein may also be used to cast other metallic materials without limitation to benefits or advantages over conventional casting techniques.

As applied to various non-limiting embodiments of the present disclosure, the centrifugal casting apparatuses, rotating assemblies, molds, and/or components thereof described herein may be comprised of a variety of metallic materials, a combination of metallic materials, ceramic materials, and/or a combination of metallic and ceramic materials. It can be appreciated that various embodiments of the present disclosure may be useful for producing, for example and without limitation, gas turbine components, turbocharger components, and/or internal combustion engine components, among many other types of components or products.

TiAl materials have traditionally been cast using static investment casting techniques. More recently, various centrifugal casting techniques, including centrifugal investment casting, have been proposed for casting TiAl materials. The above techniques, however, may allow voids to form in deleterious locations within the final cast pieces and therefore may increase production costs, limit mechanical properties, and/or impair structural characteristics of the final cast pieces. These techniques are also limited in both the number of cavities and castings per cavity. FIG. 1 illustrates a semi-schematic of a conventional centrifugal casting device 2. The device 2 generally requires supplying molten material from a material supply source "S" to a sprue chamber 4 positioned near a rotation axis "R," about which the device 2 rotates during operation. The device 2 employs indirect gating, which requires routing the molten material (shown as hatched lines) through a runner system 6 to a series of gates 8 positioned at entrances of respective mold cavities 10. Indirect gating feeds molten material to cavities in a direction other than aligned with the direction of centrifugal force "F," such as vertically, as shown in FIG. 1, or in the direction opposite to the centrifugal force, as described in U.S. Patent Application Publication US 2012/0207611 A1, for example. As such, molten material must travel an increased radial distance along various runners 6 to reach additional vertical gating components 8 that must also be traveled before reaching the entry port of the casting cavity 10. The various runners 6, and often the vertical gating components 8, are not in-line with the cast part. Thus, the molten material must enter the casting cavity 10 counter to the centrifugal force. The cross-section of the casting cavity 10 is also larger than the various runners 6, gating 8, and entry port. Thus, in addition to reducing yield due to runner loss, the device 2 is unable to adequately control shrinkage porosity and is susceptible to premature solidification, poor mold fill, and molten material starvation.

Direct gating differs from indirect gating in that the molten material is fed to the cavity generally in the direction of centrifugal force. Direct gating is not used in conventional centrifugal casting devices because indirect gating may reduce turbulence in the mold.

Referring to FIG. 2, illustrating a simplified semi-schematic depiction of certain components of one non-limiting embodiment of a centrifugal casting apparatus according to the present disclosure, a rotating assembly 12 of a centrifugal casting apparatus may be configured with a direct gating system that reduces yield loss and uses centrifugal force to control shrinkage porosity for production of dense castings. For example, in various non-limiting embodiments, a molten material source "M" may supply molten material (shown generally as hatched lines) to a sprue chamber 14 positioned on or adjacent to an axis of rotation "R" for the rotatable assembly 12. A series of gates 16a-16f, each coupled to a stacked mold cavity 18a-18f, may couple to the sprue chamber 14 to deliver molten material to the cavities 18a-18f generally in the direction of centrifugal force "F". In operation, for example, a vacuum arc remelting (VAR) melter (shown generally as molten material supply) may be used to produce a superheated melt of molten material that may be poured from the crucible through a funnel positioned above the sprue chamber 14. The superheated molten material may enter the sprue chamber 14 and begin filling the cavities 18a-18f through the adjacent gates 16a-16f until all the cavities 18a-18f are filled. According to various non-limiting embodiments, the gates 16a-16f coupled to the stacked cavities 18a-18f may be bathed in liquid molten material during at least one period of mold filling. For example, the sprue chamber 14 may be filled with superheated molten material such that all gates 16a-16f are completely submerged. In various non-limiting embodiments, one or more cavities 18a-18f are dimensioned to form multiple final pieces. For example, a gate 16a-16f may be coupled to a cavity 18a-18f dimensioned to produce a casting comprising a plurality of final pieces. In certain non-limiting embodiments, the cast pieces may be aligned along the casting cavity 18a-18f thereby increasing the number of castings that may be produced per gate.

Conventional centrifugal casting gating designs feed molten material to cavities through restricted paths, often including distinct choke points. For example, the diameter or cross-sectional area of the gates 8 in the device 2 shown in FIG. 1 are greater than the diameter or cross-sectional area of the respective casting cavities 10 attached to each gate 8. In contrast, as shown in FIG. 2, various non-limiting embodiments of the disclosed centrifugal casting apparatuses 12 may include gates 16a-16f comprising diameters or cross-sectional areas greater than those of the cavity 18a-18f or casting. For example, in some non-limiting embodiments, a volume of a length of the gate 16a-16f is greater than a volume of an equivalent length of the cavity 18a-18f. For example, a length of the gate 16a-16f adjacent to the cavity 18a-18f may comprise a larger volume than the adjacent area of the cavity 18a-18f having an equivalent length.

Known centrifugal casting techniques for TiAl materials connect a single gate 8 to a cavity 10 to produce each final cast piece, as shown in FIG. 1. Accordingly, to produce a significant number of pieces, the diameter of the sprue chamber 4 must be relatively large, requiring the molten material to travel a substantial distance from the sprue chamber 4 to the cavities 10 as a thin molten layer. When molten material travels as a thin layer, the material may lose superheat, resulting in premature solidification, poor mold fill, and castings having poor surface finish. In contrast, as shown in FIG. 2, the rotatable assembly 12 may employ direct gating to supply

molten material to a plurality of stacked cavities **18a-18f** in the general direction of centrifugal force "F." Stacked cavities **18a-18f** may increase the number of castings that may be produced per pour while also reducing the distance that the molten material must travel to reach the mold cavities **18a-18f**. For example, compared to conventional centrifugal casting devices with the same number of gates, the rotatable assembly **12** may comprise a sprue chamber **14** having a reduced diameter. Beneficially, the per gate **16a-16f** volume of molten material may be reduced, and the proximity of the volume of the molten material in the reduced diameter sprue chamber **14** may promote superheat retention. This may maintain fluidity of the molten material to prevent misruns or premature solidification that may obstruct the supply of molten material in the sprue chamber **14** from reaching the solidifying castings. Consequently, runner yield loss may be reduced, product yield may be increased, and surface finish may be improved.

In various non-limiting embodiments, the rotatable assembly **12** comprises mold designs which may control the amount and location of shrinkage porosity such that it may be internalized to the material. The internalized porosity may then be removed through subsequent thermo-mechanical processing. In certain non-limiting embodiments, molds may be fabricated from materials comprising metallic materials, such as iron and iron alloys, e.g., steels, including semi-metallic materials such as graphite. According to one non-limiting embodiment, molds fabricated from such materials may comprise permanent casting molds, e.g., generally reusable casting molds. In various non-limiting embodiments, molds fabricated from the above materials may also reduce or eliminate contamination of the cast product by entrapped oxides. For example, molds used in investment casting are typically made of oxides. During casting, however, the oxide particles making up the mold invariably become entrapped in the investment cast product. The entrapped particles may subsequently react with the material of the cast product and provide a potential fatigue initiation site. Investment casting molds may be engineered to be inert to molten TiAl or the particular alloy being cast, and various chemical and machining methods may be available to partially remove the entrapped particles. Nevertheless, particle entrapment is unavoidable and the above stopgaps are not ideal, especially for castings used to fabricate end products intended for service in high temperature, high stress environments, such as turbines. In addition to reducing or eliminating contamination of the final product by entrapped oxides, molds comprising metallic materials may reduce or eliminate risk of contamination of the recycle loop due to entrapped oxides in scrap. For example, as described above, investment castings often include entrapped oxides and, therefore, scrap, e.g., revert, from investment castings may similarly include entrapped oxides. Consequently, products cast using this recycled scrap may also be contaminated with the entrapped oxides. However, scrap from castings produced in molds fabricated from the above metallic materials, do not have a potential for such inclusions and therefore may be recycled without risk associated with contamination of the recycling loop. Consequently, extensive cleaning of scrap before recycling may not be necessary, thereby saving time and reducing costs. Despite the above benefits, it is also contemplated that some embodiments may comprise molds fabricated with other materials. For example, in various non-limiting embodiments, molds may comprise expendable centrifugal casting molds. Such molds may be fabricated from expendable materials such as sand or oxides, for example.

In certain non-limiting embodiments, molds may be structured to control the solidification process by controlling the

cooling rate of regions of the molten material. For example, molds may include insulation features configured to limit the amount and/or rate of thermal energy extraction from the molten material. Insulation features may generally comprise structural or material features associated with the mold and may be configured to modify the heat capacity of a region of the mold and/or rate of heat transfer from the molten material to the mold. In one non-limiting embodiment, the rate of heat transfer from the molten material may be at least partially controlled by the shape of the mold. For example, the thickness of one or more regions of the mold may be increased or reduced to increase or reduce the heat capacity of the region. In one non-limiting embodiment, the rate and/or amount of thermal energy that may be extracted by the mold may be controlled by the density or mass of a region of the mold. For example, in various non-limiting embodiments, one or more pockets (see, e.g., FIG. 9, **332a**, **338a**) may be defined in a wall or face of the mold adjacent to the cavity **18a-18f** to reduce the rate of heat transfer from the molten material. In various non-limiting embodiments, pockets may be enclosed, open, evacuated, or comprise a gas or material positioned in the pocket.

In various non-limiting embodiments, molds may be structured to control heat extraction from the molten material and, hence, control cooling of the material. For example, as introduced above, in certain non-limiting embodiments, a mold may comprise insulation features configured to differentially insulate one or more portions of a cavity **18a-18f**. Differential insulation features may beneficially modify the rate of cooling along one or more regions of the mold to, for example, control solidification of the molten material. For example, mold regions adjacent to the cavity **18a-18f** may be structured such that molten material undergoes directional solidification. In one aspect, molds may be configured to modify cooling such that solidification is directional, e.g., generally toward the sprue chamber **14** or in a direction opposed to the centrifugal force. In this way, the mold may establish a solidification front within the cavity **18a-18f** that generally progresses toward the gate **16a-16f** and the sprue chamber **14**. Thus, the centrifugal force generated by the rotation of the apparatus **12** may generally be opposed to the direction of solidification. For example, in certain non-limiting embodiments, molten material may be supplied to the solidification front to compensate for the shrinkage porosity. Additionally, casting pressure generated by the centrifugal force may force molten metal between dendrites forming near the solidification front to, for example, reduce molten material starvation and minimized shrinkage porosity. Consequently, in various non-limiting embodiments, the disclosed apparatuses and methods may avoid molten material starvation and overcome dendrite exclusion to produce denser castings having reduced shrinkage porosity compared to castings produced by conventional stationary and centrifugal casting techniques.

In various non-limiting embodiments, delivery of the supply of molten metallic material to the cavities **18a-18f** is in-line with the cavities and the centrifugal force. For example, in one non-limiting embodiment, the cavities **18a-18f** are coupled to the sprue chamber **14** via gates **16a-16f** disposed between the sprue chamber **14** and the cavities **18a-18f**. Various dimensions of the gates **16a-16f** may be larger than corresponding dimensions of the cavities **18a-18f**. The gates **16a-16f** may further be in-line with both the cavities **18a-18f** and the supply of molten metallic material in the sprue chamber **14**, e.g., comprising a path generally in-line with the centrifugal force such that molten material may be accelerated toward and into the cavities **18a-18f** by the centrifugal force. As a result, the sprue chamber **14** may act as a

central riser for all the gates 16a-16f attached to it. In various non-limiting embodiments, this may eliminate the need for additional risers that may or may not be in-line with the cavities. Thus, such synergy between equipment design, volume of molten material, and available casting area may beneficially provide additional space for additional castings. For example, as stated above, multiple pieces may be cast within a single casting cavity 18a-18f.

FIGS. 3-5 illustrate a centrifugal casting apparatus comprising a rotatable assembly 20 according to various non-limiting embodiments. The rotatable assembly 20 comprises a first mold 22 and a second mold 24 positioned on a rotatable table 26. A sprue chamber 28 is defined by first and second sprue sections 30a, 30b and respective front faces 32a, 32b of the first and second molds 22, 24. A first end 36 of the sprue chamber 28 is positioned on the table 26 about the rotation axis. A second end 38 of the sprue chamber 28 is configured to receive a supply of molten metallic material, e.g., from a crucible positioned above the sprue chamber 28. The first and second sprue sections 30a, 30b are configured for sealing engagement with the first and second molds 22, 24 and table 26 to seal the sprue chamber 28. While the illustrated sprue chamber 28 is shown as comprising a generally cylindrical cross-section, in various non-limiting embodiments, the sprue chamber 28 may comprise irregular or regular dimensions such as triangular, square, rectangular, octagonal, or other cross-sections. In various non-limiting embodiments, the molten material may be supplied to the sprue chamber 28 via gravity, pressure, vacuum, or a combination thereof. For example, according to one non-limiting embodiment, the centrifugal casting apparatus 20 may comprise a vacuum arc remelting device (not shown) for generating a molten metallic material supply that may be poured into the sprue chamber 28.

A containment ring 40 is positioned adjacent to the first end 36 of the sprue chamber 28 and is structured to retain molten material within the sprue chamber 28. For example, in one non-limiting embodiment, the containment ring 40 comprises an extension to the sprue chamber 28, thereby increasing the volume of the sprue chamber 28 and/or the distance molten material must travel to exit the top end of the sprue chamber 28. The containment ring 40 defines a central diameter through which molten material may be supplied to the sprue chamber 28. The central diameter of the containment ring 40 is reduced relative to the diameter of the sprue chamber 28 such that the containment ring 28 forms an internal overhang 42 within the sprue chamber 28 to improve containment of the molten material. For example, in various non-limiting embodiments, the containment ring 40 may limit molten material from splashing or flowing out of the sprue chamber 28 during pouring and/or rotation. The containment ring 40 further defines an outer diameter comprising an external overhang 44 with respect to the sprue sections 30a, 30b. In the illustrated non-limiting embodiment, the top surface 46 of the containment ring 40 extends outward with respect to the rotation axis, beyond the sprue chamber 28, to thereby catch molten material about its top surface 46 that may splash out of the sprue chamber 28 during operation.

According to various non-limiting embodiments, the second end 38 of the sprue is coupled to the table 26 via a wedge 48, as shown most clearly in FIG. 4, providing a partially exploded view of the rotating assembly 20 showing the table 26, wedge 48, and containment ring 40 in cross-section taken along line 5-5 and in the direction of the arrows in FIG. 3. The wedge 48 may form a base 47 of the sprue chamber 28 and be fixed to the rotation axis of the rotatable assembly 20. The illustrated wedge 48 is fixed to the rotation axis via the table

26 through a wedge fitting 50 defined in the table 26. The wedge 48 may further comprise one or more fittings configured for sealing engagement with the sprue sections 30a, 30b and/or molds 22, 24. For example, in various non-limiting embodiments, the wedge 48 comprises a flange fitting 50 for sealing engagement with components of the rotatable assembly 20. The wedge 48 defines two notches 52a, 52b configured for engagement with slots 54a, 54b, which are defined in the first and second molds 22, 24, respectively. In certain non-limiting embodiments, the wedge 48 may be susceptible to mechanical deterioration and, therefore, may comprise a separate, e.g., modular, component that may be replaceable if needed. Similarly, in certain non-limiting embodiments the wedge 48 may comprise various attachment designs such that the wedge 48 may be used to modify or retrofit centrifugal casting apparatuses for use according to various non-limiting embodiments disclosed herein.

The first and second molds 22, 24 are each coupled to the first and second sprue sections 30a, 30b and extend generally radially from the rotation axis. Each mold 22, 24 comprises a front face 32a, 32b and an end face 56a, 56b. The front face 32a, 32b is positioned along the sprue chamber 28 and defines entrances to the gates 60a, 60b. As shown in FIG. 5, the first and second molds 22, 24 each comprise first and second modular sections 64a,b, 66a,b, respectively, that may be separated by removing a series of bolts 68 from bolt slots 70 defined in the molds 22, 24 or by other known attachment and detachment methods. Each mold 22, 24 further includes six stacked cavities 72a, 72b. Each cavity 72a, 72b is defined by a sidewall 76a, 76b and a back wall 80a, 80b. The entrance to each cavity 72a, 72b comprises a material supply port 84a, 84b in fluid communication with the sprue chamber 28 through the gate 58a, 58b that is positioned between the cavity 72a, 72b and the sprue chamber 28. While the first and second molds 22, 24 are illustrated as defining both the stacked cavities 72a, 72b and the respective coupled gates 60a, 60b, according to various non-limiting embodiments, the gates 60a, 60b may be independent structures with respect to the cavities 72a, 72b. For example, the gates 60a, 60b may be engagable with cavities 72a, 72b and/or insertable through or unitary with a sprue or sections thereof 30a, 30b.

According to various non-limiting embodiments, the gates 60a, 60b comprise a diameter and average cross-sectional area greater than the diameter and average cross-sectional area of the cavities 72a, 72b. For example, the diameter and cross-sectional area of each gate 60a, 60b adjacent to the material supply port 84a, 84b is greater than the diameter and cross-sectional area of the adjacent material supply port 84a, 84b. In various non-limiting embodiments, a volume of a gate 60a, 60b is greater than a volume of an equal length of a cavity 72a, 72b adjacent to the gate 60a, 60b. It is to be appreciated that while six stacked cavities 72a, 72b are shown, unless expressly stated otherwise, the present disclosure is not limited to stacked cavities or any specific number of cavities associated with each mold. For example, in various non-limiting embodiments, a mold may define only a single cavity. Similarly, while only two molds 22, 24 are shown in FIGS. 3-5, it is to be understood that the present disclosure and the embodiments disclosed herein are not limited by the number of molds illustrated. Indeed, in various instances, a rotatable assembly comprises a modular design wherein the number and design of the molds may be modified as needed. For example, when fewer castings are desired, certain molds may be removed to suit the application.

In certain non-limiting embodiments, the first and second molds 22, 24 may be structured to control heat extraction from the molten metallic material and, hence, control cooling

of the material. For example, the first and second molds 22, 24 may comprise various insulation features configured to produce directional solidification of the material toward the rotation axis. The thickness of the back walls 80a, 80b may be greater than the thickness of the sidewalls 76a, 76b. Thus, heat transfer from the molten material to the molds 22, 24 may be controlled by the heat capacity of the walls 76a, 76b, 80a, 80b defining each cavity 72a, 72b. For example, differential insulation features of the molds 22, 24 may include increased heat transfer at the back wall 80a, 80b compared to heat transfer at the sidewall 76a, 76b or region thereof. Accordingly, material adjacent to the back walls 80a, 80b may begin to solidify before material positioned adjacent to the gates 60a, 60b. In this way, a solidification front may generally progress within each of the stacked cavities 72a, 72b from the back wall 80a, 80b toward the gate 60a, 60b and sprue chamber 28. In addition to establishing a solidification front, in various non-limiting embodiments, the centrifugal casting force generated by the rotation of the molds 22, 24 about the rotation axis is generally opposed to the direction of solidification, thereby preventing molten material starvation and dendrite exclusion that may result in uncontrolled porosity in castings produced by conventional stationary and centrifugal casting techniques. For example, the sprue chamber 28, gates 60a, 60b, and portions of the cavities 72a, 72b located ahead of the solidification front may act as a reservoir to forcefully supply molten material to the solidification front to produce dense castings having controlled shrinkage porosity.

In certain non-limiting embodiments, the first and second molds 22, 24 are structured to control heat transfer from the molten metallic material to the mold while not detrimentally decreasing the cooling rate of the material. For example, the first and second molds 22, 24 may be structured to provide various levels of control over the solidification process while also providing increased solidification rates. As those having skill in the art will appreciate, an increased cooling rate may favorably decrease grain size, thereby benefiting mechanical properties of the casting at room temperature. Such an increased cooling rate in conventional designs, however, is difficult to control and results in uncontrolled shrinkage porosity. In contrast, in various non-limiting embodiments, the first and second molds 22, 24 are permanent molds and/or are fabricated from materials including metallic materials to provide increased solidification rates due to a high thermal conductivity that may be associated with the mold material, to thereby promote decreased grain size. For example, in one non-limiting embodiment, the first and second molds 22, 24 comprise a permanent steel mold. The first and second molds 22, 24 may also be structured to promote directional solidification, as described above, without sacrificing grain size due to, for example, a retarded cooling rate. That is, while certain portions of the molds 22, 24 may be differentially thermally insulated relative to other portions of the mold 22, 24, the overall cooling rate may be relatively fast. For example, the first and second molds may be configured to promote a differential cooling rate that is tightly defined, e.g., optimized to promote formation of a solidification front that rapidly progresses from the back wall 80a, 80b toward the sprue chamber 28.

While not shown in FIGS. 3-5, in various non-limiting embodiments, the mold walls 76a, 76b, 80a, 80b may comprise multiple insulation features, such as pockets or other insulation features. For example, mold walls 76a, 76b, 80a, 80b may comprise multiple materials having various heat capacities and densities to modulate heat transfer from the molten material. For example, a pocket or void may be defined in a wall adjacent to a cavity. The reduced mass of the

wall may limit the ability of the wall to extract heat from the molten material. Accordingly, in various non-limiting embodiments, walls defining pockets may have limited heat capacity thereby limiting the amount of thermal energy that the walls may absorb before thermal saturation is reduced. Accordingly, such walls may insulate the cavity to control heat transfer from the molten metallic material. In various non-limiting embodiments, a cavity 72a, 72b may be defined by a back wall 80a, 80b and a sidewall 76a, 76b comprising a first and second sidewall portion. In some instances, the first and second sidewall portions may comprise the same thickness, while in other instances, the thicknesses of the first and second sidewall portions may be different. For example, when a first sidewall portion is disposed between two cavities, the first sidewall portion may be thicker than the second sidewall portion that is adjacent to only a single cavity. Similarly, in various non-limiting embodiments, as shown in FIGS. 3-5, the molds 22, 24 may be insulated from the table 26 by a boundary layer comprising interfacing surfaces of the molds 22, 24 and the table 26.

FIG. 6 illustrates certain components of a non-limiting embodiment of a centrifugal casting apparatus comprising a rotatable assembly 100 according to various non-limiting embodiments of the present disclosure. The rotatable assembly 100 comprises eight molds 102a-102h, each positioned on a rotatable table 104. The molds 102a-102h define a generally octagonal sprue chamber 106 positioned about the rotation axis and radiate generally outward to define back faces 108a-108h. FIG. 7 illustrates a cross-section of the rotatable assembly 100, taken along line 7-7 and in the direction of the arrows in FIG. 6, and shows a vertical cross-section of six stacked cavities 110a and 110e defined by molds 102a and 102e, respectively. The molds 102a-102h each comprise a front face (only front faces 112a, 112c-112e are visible) configured for sealing engagement about the rotation axis to define the sprue chamber 106. The sprue chamber 106 extends from the table 104 to a raised containment ring 114 structured to retain molten material within the sprue chamber 106.

The sprue chamber is in fluid communication with the stacked cavities 110a, 110e at the material supply ports 116a, 116e of each of the stacked cavities 110a, 110e via respective gates 118a, 118e. The stacked cavities 110a, 110e are each defined by a sidewall 120a, 120e and a back wall 122a, 122e. For brevity, various features of the rotatable assembly 100 may be described with respect to molds 102a and 102e. It is to be appreciated, however, that in various embodiments, the descriptions apply similarly to one or more additional molds 102b-102c, 102f-102h. For example, the six stacked cavities 110c, 110d of molds 102c and 102d may also be in fluid communication with the sprue chamber 106 at material supply ports 116c and 116d via gates 118c, 118d. The gates 118a, 118e comprise a diameter and average cross-sectional area greater than the diameter and average cross-sectional area of the respective stacked cavities 110a, 110e coupled to each of the gates 118a, 118e. For example, the diameter and cross-sectional area of the gates 118a, 118e adjacent to the material supply ports 116a, 116e are greater than the diameter and cross-sectional area of the material supply ports 116a, 116e or the cavities 110c, 110d. In various non-limiting embodiments, each gate 118a, 118e defines a volume greater than a volume defined by an equal length of the cavity 110a, 110e adjacent to the gate 118a, 118e.

In operation, the rotatable assembly 100 of the centrifugal casting apparatus utilizes centrifugal forces generated by the rotation of the rotatable assembly 100 to produce castings by centrifugal casting. In one non-limiting embodiment, the cen-

trifugal casting apparatus comprises a vacuum arc remelting apparatus (not shown) configured to consume an electrode of metallic material to be supplied to a crucible, such as a water-cooled copper crucible. For example, the rotatable assembly 100 may be positioned within a vacuum environment such that when the electrode is consumed, the molten metallic material within the crucible may be supplied to the rotatable assembly 100. The rotatable assembly 100 may generally comprise the sprue chamber 106 positioned about the rotation axis and two or more stacked mold cavities 110a, 110e defined in one or more molds 102a, 102e. While not shown in detail in FIGS. 6-7, each of the stacked mold cavities 110a, 110e may be structured to form a casting comprising one or more pieces. When the molten metallic material is supplied to the sprue chamber 106, the centrifugal force generated by the rotation of the rotatable assembly 100 accelerates the molten metallic material through the gates 118a, 118e and into the casting cavities 110a, 110e. In various non-limiting embodiments, the molds 102a, 102e may be rotatable to speeds including 100 and 150 rotations per minute (RPM). More preferably, rotational speeds may be greater than 150 RPM. In general, faster rotational speeds may provide castings having improved structure. For example, compared to a rotational speed of 160 RPM, a rotational speed of 250 RPM would produce increased centrifugal force, which may reduce porosity of the cast part. In various embodiments, a relative increase in centrifugal force may allow a relative increase in a solidification rate to promote reduced grain size and/or additional margin of error with respect to controlling directional solidification.

As the molds 102a, 102e extract heat from the molten metallic material, the material begins to freeze, producing shrinkage porosity. According to various non-limiting embodiments, heat extraction may be limited by the thickness of the walls 120a, 120e, 122a, 122e of the mold. For example, in one non-limiting embodiment, the thickness of the side-walls 120a, 120e may be less than 1 inch. Accordingly, the thickness of the walls 120a, 120e, 122a, 122e may limit the ability of the mold 102a, 102e to absorb thermal energy from the molten material. As described above, in various non-limiting embodiments, the molds 102a, 102e are configured to control cooling of the material such that the material undergoes directional solidification from the back walls 122a, 122e generally toward the axis of rotation or the sprue chamber 106. The dimensions of the gates 118a, 118e leading to the cavities 110a, 110e are also large enough to prevent the supply of molten material in the sprue chamber 106 from being cut off from the shrinkage porosity. As a result, most of the porosity may be filled with molten material. When the material in the cavities 110a, 110e fully solidifies, the respective casting gates 118a, 118e also freeze, which closes off the molten material that may remain in the sprue chamber 106 from the casting cavities 110a, 110e. Accordingly, gates 118a, 118e may be fully dense upon freezing. When the solidified metallic material in the cavities 110a, 110e is sufficiently cooled to handle and no longer oxidize, the castings may be removed from the molds 102a, 102e, for example, by unbolting a first modular mold section from a second modular mold section, which may be similar to the arrangement described above with respect to modular mold sections 64a, 64b. The castings may be removed from the sprue chamber 106 at or near the position where the gates 118a, 118e meet the sprue chamber 106. Since the gates 118a, 118e are fully dense, any porosity inside the casting remains internal and may be removed by HIP, for example, to eliminate any internal porosity in the casting. When castings comprise multiple pieces, the fully dense casting may then be divided into the

final pieces by machining equipment such as saws, cutting torches, abrasive water jet, or wire electro-discharge machining apparatuses, for example.

As introduced above, in various non-limiting embodiments, the gates 118a, 118e comprise a diameter or cross-sectional area greater than the largest diameter or cross-sectional area of the cavities 110a, 110e. In certain non-limiting embodiments, the increased size of the gates 118a, 118e prevents internal porosity from reaching the sprue chamber 106. For example, a gate 118a, 118e may be fully dense upon solidification, preventing internal porosity from connecting to the sprue chamber 106 where it may later become exposed when the casting is removed from the sprue chamber 106. Thus, gates 118a, 118e may form a density barrier to contain the internal porosity such that it may be addressed by processing, such as by HIP, for example. In various non-limiting embodiments, gates 118a, 118b may form a thermal barrier between casting cavities 110a, 110e and the sprue chamber 106. For example, the cooling rate of the molten metallic material in the sprue chamber 106 may be well below the cooling rate of the molten metallic material in the cavities 110a, 110e, resulting in a substantial temperature differential between the cavities 110a, 110e and the sprue chamber 106 well after an optimal cooling period for the casting has taken place. Consequently, grain size near the sprue chamber 106 may be increased. The gates 118a, 118e disclosed herein, however, may be configured to solidify closely following the casting, e.g., when the solidification front has extended through the casting, but still before the molten metallic material in the sprue chamber 106 has solidified. According to one non-limiting aspect, the solidified gates 118a, 118b, which may also be fully dense, thereby form a thermal barrier between the sprue chamber 106 and respective casting cavities 110a, 110e.

In various non-limiting embodiments, the rotatable assembly 100 comprises a plurality of vertically stacked cavities 110a, 110e positioned about a sprue chamber 106. The sprue chamber 106 may comprise a decreased radius compared to sprue chambers of conventional centrifugal casting apparatuses that are configured to feed a comparable number of cavities. In operation, according to one non-limiting embodiment, molten material may substantially simultaneously, e.g., continuously, fill the sprue chamber 106, gates 118a, 118e, and vertical cavities 110a, 110e. For example, molten material supplied to the sprue chamber 106 may begin to simultaneously fill the sprue chamber 106, adjacent gates 118a, 118e, and vertical cavities 110a, 110e from the bottom toward the top. Thus, as the molten material is poured into the sprue chamber 106, the molten material accumulates to form an increasing molten volume in the sprue chamber 106 that may be directly fed to the adjacent gates 118a, 118e and vertical cavities 110a, 110e without loss of superheat due to excessive travel and contact with various structures of the rotatable assembly 100. Thus, in various non-limiting embodiments, the sprue chamber 106 is configured to feed all the casting cavities 110a, 110e while promoting retention of superheat. For example, in operation, the sprue chamber 106 may be dimensioned to receive a single pour of molten material that completely fills a cavity of the vertical stacks of cavities 110a, 110e. For example, in one non-limiting embodiment, the sprue chamber is dimensioned to receive a single pour of molten material that completely fills at least the bottom cavity of each of the vertical stacks of cavities 110a, 110e. The volume of the single pour is preferably sufficient to also completely fill the gates 118a, 118e and the volume of the sprue chamber 106 adjacent to the completely filled cavities 110a, 110e. Thus, the rotatable assembly 100 may be config-

## 15

ured to receive a volume of molten material that may be fed directly from the sprue chamber **106** into the cavities **110a**, **110e** without loss of superheat.

According to certain non-limiting embodiments, retaining superheat promotes production of cast pieces comprising improved surface quality. Titanium aluminide castings, for example, produced by conventional casting techniques suffer from poor surface quality. For instance, as stated above, when a thin layer of molten material must travel the radius of a large diameter sprue and subsequently climb various structures, such as sprue walls or gating, for example, to fill from the bottom of the mold cavities, the bulk of the molten material may be unable to retain superheat, resulting in poor surface quality. The poor surface quality may require producing castings several millimeters larger than the final piece so that the surface of the casting may be processed to produce a casting within the desired dimensions. In contrast, the rotatable assembly **100** may be configured to produce castings comprising improved smoothness and without surface defects commonly found in castings produced by conventional techniques. Consequently, castings may be produced with lower scrap rates and production costs.

FIG. 8 is a front view of a mold **200** according to certain non-limiting embodiments of the present disclosure. The mold **200** includes first and second modular sections **202**, **202** that define seven cavities **210**. The cavities **210** extend from a front face **212** of the mold **200** toward a back wall **214** of the mold **200** and are defined between sidewalls **216**. In certain non-limiting embodiments, the mold may be structured to control cooling of molten material such that the material undergoes directional solidification from the back walls **214** generally toward the axis of rotation or the sprue chamber, which may be proximate to the front face **212** of the mold **200**. The mold further includes gates **218** positioned adjacent to the front face **212** leading to each cavity **210a**. The gates **218** are dimensioned to prevent the supply of molten material in the sprue chamber from being cut off from the shrinkage porosity. As a result, most of the porosity may be filled with molten material to produce dense castings. For example, the gates **218** comprise a diameter or cross-sectional area greater than the largest diameter or cross-sectional area of the cavities **210**. In certain non-limiting embodiments, the increased size of the gates **218** prevents internal porosity from reaching the sprue chamber. For example, a gate **218** may be fully dense upon solidification, preventing internal porosity from connecting to the sprue chamber where it may later become exposed when the casting is removed from the sprue chamber. Thus, the gates **218** may form a density barrier to contain the internal porosity such that it may be addressed by processing, such as by HIP, for example. As described above, in various non-limiting embodiments, the gates **218** may also form a thermal barrier between the casting cavities **210** and the sprue chamber. Consequently, grain size near the sprue chamber may be reduced compared to conventional castings because the material in the gates **218** may solidify closely following the casting, e.g., when the solidification front has extended through the casting, but still before the molten metallic material in the sprue chamber has solidified. As described above, when the solidified material in the cavities **210** has sufficiently cooled, the castings may be removed from the mold **200** by separation of the first and second modular sections **202**, **202**.

FIG. 9 is a perspective view of certain components of a rotatable assembly **300** of a centrifugal casting apparatus according various non-limiting embodiments of the present disclosure. The rotatable assembly **300** comprises a sprue **302** coupled to a first mold **304** and a second mold **306**. The sprue

## 16

**302** is positioned about a rotation axis of the assembly **300** and defines a sprue chamber **308** structured to receive a supply of molten metallic material. The sprue chamber **308** comprises a generally cylindrical shape having a generally circular cross-section. The outer surface of the sprue **302** defines two slots **310a**, **310b** for receiving the molds **304**, **306**. Each mold **304**, **306** comprises first and second modular sections **312a**, **b**, **314a**, **b** attachable via bolts **316**, which are insertable through slots **318** defined in the molds **304**, **306**.

10 Each mold defines five stacked cavities, wherein two of the cavities **320a**, **322a** comprise a decreased diameter compared to three larger diameter cavities **320b**, **322b**. The decreased diameter cavities **320a**, **322a** are positioned at intervals between the three larger diameter cavities **320b**, **322b**. As can be seen, multiple diameter cavities may increase flexibility with respect to casting sizes that may be produced in a single pour. For example, time and yield loss may be reduced by consolidating pours. The stacked cavities **320a**, **320b**, **322a**, **322b** are in fluid communication with the sprue chamber **308** through respective gates **324a**, **324b**, **326a**, **326b**. Each gate **324a**, **324b**, **326a**, **326b** comprises a diameter and cross-sectional area larger than the diameter and cross-sectional area of the cavity **320a**, **320b**, **322a**, **322b** in which it is coupled. In one aspect, the increased size of the gates **324a**, **324b**, **326a**, **326b** prevents full solidification of the gates **324a**, **324b**, **326a**, **326b** until after the material in the respective cavities **320a**, **320b**, **322a**, **322b** has fully solidified. That is, at least a portion of the material in the gates **324a**, **324b**, **326a**, **326b** may retain liquidity such that it may move into and fill portions of the solidifying metallic material in the casting cavity **320a**, **320b**, **322a**, **322b**. As summarized above, in various non-limiting embodiments, gates **324a**, **324b**, **326a**, **326b** comprise an increased dimension with respect to a dimension of the cavity. For example, according to certain configurations, optimal efficiency with respect to casting volume and yield may include a gate **324a**, **324b**, **326a**, **326b** comprising a cross-sectional area greater than the cross-sectional area of the cavity **320a**, **320b**, **322a**, **322b**, for example, between 100% to 150% of the cross-sectional area 40 of the cavity **320a**, **320b**, **322a**, **322b**. Of course, in some non-limiting embodiments, gates comprising cross-sectional areas up to, for example, 400% or more of the cross-sectional area of the corresponding cavity, may also be used to produce castings having similar characteristics. Yield loss, however, 45 may increase with increasing gate dimensions. According to various configurations of certain non-limiting embodiments, optimal gate lengths may comprise 50% to 150% of the largest dimension of the cross-section of the gate. Again, such lengths are merely optimizations of certain embodiments 50 with respect to the number of castings that may be produced per volume of material supplied to the mold, and such examples are not intended to be limiting unless stated otherwise.

The first and second molds **304**, **306** are structured to 55 promote directional solidification generally toward the rotation axis or sprue chamber **308** such that centrifugal force continually presses molten material toward the solidification front of the casting to fill shrinkage porosity as it appears in order to produce a denser casting. The first and second molds **304**, **306** comprise insulation features configured to promote directional solidification toward the sprue chamber **308**. For example, the molds **304**, **306** each comprise a side face **328**, **330** defining two pockets **332a**, **b**, **334a**, **b** spaced apart and positioned proximal to the sprue **302**. The pockets are configured to reduce the heat capacity of the mold along the corresponding portion of the mold. The molds **304**, **306** further define a plurality of upper and lower pockets **336a**, **b**,

**338a,b** extending along a portion of the molds **304, 306**. The upper and lower pockets **336a,b, 338a,b** are configured to insulate adjacent portions of the mold by limiting the heat capacity and rate of heat transfer through the mold. In addition to controlling heat transfer by altering heat capacity of portions of the mold via pockets or mass of mold walls, in various non-limiting embodiments, cavities may also be arranged to assist in controlling heat transfer.

FIG. 10 illustrates a cross-section of a mold **400** for a centrifugal casting according to various non-limiting embodiments of the present disclosure. The mold **400** includes a front face **406** and two side faces **408**, although only one side face **408** is included in the cross-section. Six cavities **410** are defined within the mold **400** between respective sidewalls **412** and back walls **414**.

Each cavity **410** comprises a molten material supply port **416** adjacent to a tapered or decreasing cross-section tapered from the material supply port **416** toward the back wall **414**. In various non-limiting embodiments, the front face **406** may be configured to attach to a gate or plate, or directly to a sprue at the molten material supply port **416**. For example, in some non-limiting embodiments, a mold **400** comprises a cavity **410** defining a decreasing cross-section over a portion of its length extending from the molten material supply port **416**, which may be directly couplable to a sprue or sprue chamber. That is, the reduction in cross-section over an initial length of the cavity **410** may overcome the need for a gate. As such, castings may be produced with reduced yield loss and controlled shrinkage porosity. In various non-limiting embodiments, cavities **410** comprising decreasing cross-sections may define sidewalls **412** generally tapering in-line with the cavity **410**, e.g., generally aligned with a centerline of the cavity **410**, and may comprise a symmetrical taper with respect to adjacent sidewalls **412** of the cavities **412**. In one non-limiting embodiment, a decreasing cross-section may be generally defined along the direction of centrifugal force and/or taper in a general direction opposed to the general direction of solidification. For example, in one non-limiting embodiment, a cavity defines a cross-section, such as a tapered section, that generally tapers away from the molten material supply port, e.g., toward a back wall **414** of the cavity **410**.

In one non-limiting embodiment, the cavity **410** defines a decreasing cross-section comprising a tapered section that includes a first cross-section and a second cross-section. The second cross-section is less than the first cross-section and is located a greater distance from the rotation axis than the first cross-section. In operation, a solidification front may be formed and directionally advance generally from the back wall **414** toward first cross-section and the molten material supply port **416**. Solidification of the material along the solidification front may result in dendrite formation within the solidifying material. According to various non-limiting embodiments, at least a portion of the molten material in front of the solidification front may remain molten for a period of time during which the material located at or near the second cross-section is subject to cooling and hence shrinkage. In this way, the molten material in front of the solidification front, e.g., at or near the first cross-section, may be accelerated by the centrifugal force such that it moves into and/or between the forming dendrites to fill shrinkage porosity as it arises to avoid formation of significant voids and thereby produce a dense casting. In this way, the portions of the mold in front of the solidification front, e.g., located more proximate to the sprue chamber, may act as a riser for the cavity **410**. In various non-limiting embodiments, cavities may comprise multiple tapered sections. In certain non-limiting

embodiments, the decreasing cross-section may prevent internal porosity from reaching the sprue chamber. In one non-limiting embodiment, the decreasing cross-section may form a density barrier to contain internal porosity such that it may be addressed by processing, such as by HIP, for example. For example, in use, at least a portion of the decreasing cross-section at or adjacent to the largest cross-section of the decreasing cross-section, e.g., at or adjacent to the molten material supply port **416**, may be fully dense upon solidification, thereby preventing internal porosity from connecting to the sprue chamber where it may later become exposed when the casting is removed from the sprue chamber.

The mold **400** further includes insulation features comprising a plurality of pockets **418** defined in the sidewalls **412** defining the cavities **410**. In various non-limiting embodiments, the sidewalls **412** of the mold **400** may also or alternatively comprise insulation features such as pockets similar to those illustrated in FIG. 9. For example, pockets defined in one or both of the sidewalls **412** may be structured to alter the heat capacity of the mold along a lateral portion of the sidewall **412**. The pockets **418** are dimensioned and positioned to promote directional solidification from the back wall **414** toward the front face **406**. As with other various non-limiting embodiments, the particular length, area, and/or position of the pockets **418** may be adjusted to suit specific parameters or pour conditions, e.g., pour temperature, mold volume, phase transformation characteristics of the metallic material, mold composition, cavity dimensions, number and proximity of cavities, and/or number and proximity of molds. In certain non-limiting embodiments, the mold may comprise two or more modular sections. The modular sections, for example, may comprise horizontal, vertical, angled, or slotted cross-sections to assist in removal of castings.

FIG. 11 illustrates a mold **500** for use in a centrifugal casting apparatus according to various non-limiting embodiments of the present disclosure. The mold **500** comprises a front face **502**, a back face **504**, an upper face **506**, a lower face **508**, a first side face **510**, and a second side face **512**. Four stacked cavities **514a-514d** extend into the mold **500** from the front face **502** toward the back face **504**. Each cavity **514a-514d** is defined by a sidewall **516**. The mold **500** further defines insulation features comprising a plurality of pockets **526** positioned about each cavity **514a-514d**. As shown, the pockets **526** are equally spaced about the cavities **514a-514d**. In certain non-limiting embodiments, however, the number, spacing, and/or dimensions of one or more pockets **526** may be different. While not shown in FIGS. 11-15, the mold **500** may further comprise gate sections at or near portions of the cavities **514a-514d** adjacent to the front face **502** of the mold **500**. Gate sections may be defined in the mold **500** or may be attachable, for example, to the front face **502**.

FIGS. 12-15 illustrate cross-sections of the mold **500** along the cavities **514a-514d** according to various non-limiting embodiments of the present disclosure. FIGS. 12-13 depict cross-sections along the first and second cavities **514a, 514b**, respectively. The cavities **514a, 514b** extend from the front face **502** of the mold **500** to respective back walls **528**, which are positioned adjacent to the back face **504**. The cavities **514a, 514b** extend substantially perpendicular to a plane defined by the front face **502**. In operation, e.g., when the mold **500** is rotated about an axis of rotation, the angular velocity of the cavities **514a, 514b** is substantially perpendicular to a radius extending from the center of rotation. The pockets **526** extend substantially parallel to the cavities **514a, 514b** and are configured to reduce the heat capacity of the sidewall adjacent to the cavities **514a, 514b** and limit the rate of heat transfer from the molten material to the mold **500**. In

the illustrated non-limiting embodiment, the back walls 528 represent a complete condition of thermal heat extraction from the molten material to the mold. Accordingly, rate of heat extraction from the molten material may be differentially controlled to promote directional solidification generally from the back walls 528 toward the front face. As stated above, when the mold 500 is rotated, centrifugal force may direct molten material toward and against the solidification front to reduce shrinkage porosity.

FIGS. 14-15 illustrate variations in arrangements of the cavities and show radially offset cavities. FIG. 14 illustrates a cross-section of the mold 500 along the third cavity 514c, which extends from the front face 502 toward the back wall 528. The pockets 526 extend substantially parallel to the cavity 514c and are configured to reduce the rate of heat transfer from the molten material to the mold 500, as described above. The cavity 514c is radially offset and defines about a 15 degree angle with respect to the second cavity 514b. FIG. 15 illustrates a cross-section of the mold 500 along the fourth cavity 514d, which extends from the front face 502 toward the back wall 528. The pockets 526 extend substantially parallel to the cavity 514d and are configured to reduce the rate of heat transfer from the molten material to the mold 500, as described above. The cavity is radially offset and defines about a 15 degree angle with respect to the second cavity 514b and about a 30 degree angle with respect to the third cavity 514c. Thus, the third and fourth cavities 514a, 514b may be radially offset, e.g., the angular velocity of a centerline of the cavity is not perpendicular to a radius originating at the center of rotation. However, as above, the back walls 528 represent a complete condition of thermal heat extraction from the molten material to the mold. Accordingly, rate of heat extraction from the material may be differentially controlled to promote directional solidification from the back walls 528 toward the front face. As stated above, when the mold 500 is rotated, centrifugal force will direct molten metallic material toward and against the solidification front to reduce shrinkage porosity.

According to certain non-limiting embodiments of the present disclosure, a tapered gate structure can be applied to various embodiments of the centrifugal casting apparatuses, rotatable assemblies, and/or molds described herein. With reference to FIG. 16, for example, a gate 602 communicates with an entry port 604 of at least one cavity 606 of a mold 608. The gate 602 may include a tapered portion 610 structured to be adjacent to the entry port 604 of the cavity. The tapered portion 610 may include one or more tapered sub-portions 610a, 610b, 610c, or may be embodied as a single tapered portion, for example. In certain embodiments, the tapered portion 610 may be embodied as an arc, for example, or another type of geometric configuration. As shown, the tapered portion 610 may extend around substantially the entire cross-sectional area of the gate 602 adjacent to the entry port 604 of the cavity 606, for example. In other embodiments, the tapered portion 610 may extend around less than the entire cross-sectional area of the portion of the gate 602 adjacent to the entry port 604 of the cavity 606. In one non-limiting example, the tapered portion 610, or sub-portions 610a, 610b, 610c thereof, may define an angle relative to a center line of a product or component cast in the mold 608, for example, wherein the defined taper angle may be in the range of greater than zero degrees to 90 degrees.

In various embodiments, an actual or average cross-sectional area defined by the tapered portion 610 of the gate 602 may be more than a cross-sectional area defined by the entry port 604 of the cavity 606 of the mold 608. In a preferred embodiment, the actual or average cross-sectional area

defined by the tapered portion 610 of the gate 602 may be in the range of greater than 100% to 150% of the cross-sectional area defined by the entry port 604 of the cavity 606. In one non-limiting example previously described above with respect to FIGS. 3-5, the diameter and cross-sectional area of each gate 60a, 60b adjacent to the material supply port 84a, 84b can be greater than the diameter and cross-sectional area of the adjacent material supply port 84a, 84b.

The inventors have discovered that a number of factors may 10 determine the structure of the tapered portion 610 of the gate 602, and/or the selection of the ratio of the cross-sectional area defined by the tapered portion 610 of the gate 602 to the cross-sectional area defined by the entry port 604 of the cavity 606. Such selection factors may include, without limitation, 15 the type of molten material being cast in the mold 608, the type of material which comprises the mold 608, desired thermodynamic characteristics such as heating and cooling rates or heat distribution, the geometry of the component being cast in the mold 608, the amount of product material sacrificed or 20 yield loss that may occur as a result of using the tapered portion 610, and/or other selection criteria. In certain embodiments, selection of an angle for a tapered portion of a gate may be responsive to desired or required fluid liquid movement characteristics.

With reference to FIG. 16A, in certain non-limiting embodiments of the present disclosure, a gate 632 can be structured with a generally trapezoidal shape, for example, for operative association with a cavity 634 of a mold. In certain embodiments, the gate 632 may be structured with 30 tapered portions 636, 638 at an included angle of 20 degrees or less, for example. It can be seen that tapered portions 636, 638 of the gate 632 may extend along part or substantially the entire distance 640 of a longitudinal axis of the gate 632. The distance 640 may represent the distance from a sprue chamber (not shown) of a casting apparatus, for example, to the entry port of the cavity 634. In certain embodiments, an actual or average cross-sectional area defined within the tapered portions 636, 638 of the gate 632 may be in the range of 35 greater than 100% to 150% of the cross-sectional area defined by the entry port of the cavity 634. In other non-limiting embodiments, the gate 632 may be structured as a generally rectangular or generally square geometry, for example, among other types of shapes. It can be seen that the gate 632 may be structured to provide a descending cross-section moving 40 from the sprue chamber toward the entry port of the cavity 634. Also, in certain non-limiting embodiments, the cavity 634 itself may be tapered at a taper angle (see, e.g., FIG. 22).

With reference to FIG. 17, in accordance with certain non-limiting embodiments of the present disclosure, a mold 652 may be structured with one or more cavities 654 having an extended gate 656, as shown. In practice, operating a casting apparatus using this mold 652 can produce components or parts that can be divided or cut into sub-components or sub-parts, for example, through post-casting processing. For 50 example, a component produced in the cavity 654 may be later sub-divided into multiple sub-components. In one non-limiting example, a component or part produced in the cavity 654 may yield twelve sub-components, wherein each such sub-component has an aspect ratio in the range of two to three. In this example, and for illustration purposes only, each such 55 sub-component might be produced with a thickness of 55 mm and height of 150 mm, resulting in an aspect ratio of about 2.7. In another non-limiting example, a component or sub-component could be produced with an aspect ratio of about 7.7 or more. FIG. 18 illustrates an example of a mold 662 structured for casting a single component from which multiple sub-components having an aspect ratio of about 7.7, for example,

can be produced. In the example shown, a gate 664 of the mold may include one or more tapered portions 666, 668, defining an approximate taper angle which may be in the range of approximately four to six degrees, for example. It can also be seen in this particular embodiment that the mold 662 includes only a single cavity 670.

In certain non-limiting embodiments, the mold 652 may be structured with one or more slots 653, 655, 657, into which one or more gate side walls (such as side wall 659) may be removably inserted. The gate side wall 659 may be comprised of a variety of different materials and may be comprised of the same or different material as the material comprising the mold 652. In one non-limiting embodiment, the side wall 659 may be embodied as a metallic insert, for example; in other embodiments, the side wall 659 may be embodied as a semi-metallic or non-metallic component. For example, use of such side walls 659 allows for control of heat transfer by selecting materials to fill the slots 653, 655, 657 which can contain lower thermal conductivity, heat capacity, or a combination thereof, in comparison to other materials that may be used within the mold 652. The slots 653, 655, 657 may be formed in round or square geometries, for example, among other potential structural shapes.

The inventors have discovered that casting a component (e.g., a plate) in the mold 652 by using an extended gate 656 as shown in FIG. 17, for example, or by using a single cavity 670 in the mold 662 as shown in FIG. 18, for example, can in many cases reduce the as-cast porosity of the product. Heat extraction can be further reduced by eliminating contact surfaces between the molten material and the mold cavity. Such a reduction in heat extraction enhances a directed solidification front. In addition, there may be reduced yield loss for the product due to a diminished need to perform peripheral machining, for example, of the cast products. For example, it can be seen that the ratio of the surface area of the cast product in the cavity 654 to the surface area of the peripheral edges of the cast product in cavity 654 is larger in comparison to components that may be cast in other cavities 672, 674, 676 of the mold 652. In certain non-limiting embodiments, one or more of the cavities 654, 672, 674, 676 may also include an operatively associated gate 656, 684, 686, 688 structured with one or more tapered portions 692, 694, 696, 698 (as described above).

In accordance with certain non-limiting embodiments of the present disclosure, FIG. 19 illustrates an example of a mold 702 wherein two cavities 704, 706 of the mold 702 share a common gate 708 in communication with both of the cavities 704, 706. The common gate 708 may be employed in various casting processes subject to consideration of factors such as, without limitation, the type of molten material being cast in the mold 702, the type of material which comprises the mold 702, desired thermodynamic characteristics such as heating and cooling rates or heat distribution, the geometry of the component being cast in the cavities 704, 706 of the mold 702, and/or other criteria. In certain non-limiting embodiments, one or more of the cavities 704, 706, 712, 714, 716 may include a gate 708, 722, 724, 726 structured with one or more tapered portions 732, 734, 736, 738 (as described above).

In certain non-limiting embodiments, the mold 702 may be structured with one or more slots 752, 754, 756 into which one or more gate side walls (such as side wall 758) may be removably inserted. The gate side wall 758 may be comprised of a variety of different materials and may be comprised of the same or different material as the material comprising the mold 702. In one non-limiting embodiment, the side wall 758 may be embodied as a metallic insert, for example; in other

embodiments, the side wall 758 may be embodied as a semi-metallic or non-metallic component. For example, use of such side walls 758 allows for control of heat transfer by selecting materials to fill the slots 752, 754, 756 which can contain lower thermal conductivity, heat capacity, or a combination thereof, in comparison to other materials that may be used within the mold 702. The slots 752, 754, 756 may be formed in round or square geometries, for example, among other potential structural shapes.

FIGS. 20-21 illustrate an example of a centrifugal casting apparatus 802 structured in accordance with certain non-limiting embodiments of the present disclosure. The casting apparatus 802 includes multiple molds 804, 806, 808, 810, 812, 814, 818 extending radially outwardly from a centrally positioned sprue chamber 820. In various embodiments, one or more of the molds 804-818 may be comprised of multiple types of materials. For example a main body portion 832 of mold 804 may be composed of a first type of material; and a back wall 834 of the mold 804 may be composed of a second type of material, wherein the first type of material is different than the second type of material. The materials may be different kinds of metallic or ceramic materials, for example. In certain embodiments, the back wall 834 may be structured to be removable or detachable from the main body portion 832 of the mold 804, such as by use of bolts, screws, or other conventional fasteners. In this manner, one type of material can be exchanged for another type of material for one or more of the molds 804-818, subject to considerations such as casting process objectives, component geometry, or thermodynamic factors such as material heat transfer qualities or heat distribution criteria.

In certain non-limiting embodiments, one or more of the molds 804-818 of the casting apparatus 802 of FIG. 20, for example, may be structured in accordance with the mold 852 illustrated in FIG. 22, for example. The mold 852 may include a main body portion 854 and a separate back wall portion 856 which can be detached or attached to the main body portion 854, as desired. In addition, one or more of the cavities 862, 864, 866, 868, 870, 872 included within the mold 852 may be structured to be tapered at a taper angle from the front face 882 of the mold 852 toward the back wall portion 856. It can be appreciated that during operation of the casting apparatus 802, concentrating more mold 852 material and less cavity 862-872 portions away from the front face 882 toward the back wall portion 856, for example, can create more of a heat sink effect adjacent to the back wall portion 856. In this manner, the overall thermodynamic behavior of the mold 852 can be adjusted in response to the amount of taper structured into the cavities 862-872, the amount of back wall portion 856 material added to or detached from the mold 852, and/or the type of materials respectively comprising the main body portion 854 and the back wall portion 856, among other factors.

In accordance with certain non-limiting embodiments described herein, it can be appreciated that a gate structure and a cavity for forming a product or component may both have one or more tapered portions within the same mold. In one example, a tapered cavity structure as shown in FIG. 22, for example, can be coupled with one or more of the various tapered gate structures or geometric gate structures described herein.

It is appreciated that certain features of the centrifugal casting apparatuses and methods described herein are described in terms of illustrated embodiments. For example, for brevity and ease of understanding, only a limited number of variations with respect to the number and arrangement of molds and cavities are illustrated. As will become apparent to one of ordinary skill in the art after reading this document, the

23

illustrated embodiments and their various alternatives may be implemented without confinement to the illustrated examples. The present disclosure is also not limited to the illustrated cavity or mold arrangements. For example, in various embodiments, molds may comprise multiple vertical stacks of cavities. Stacked cavities may comprise molds comprising multiple rows of stacked cavities. Stacked cavities may also comprise one or more cavities radially offset from the center of rotation. For example, a mold may comprise a stack of cavities wherein all the cavities are radially offset. In some non-limiting embodiments, stacked cavities may comprise multiple rows of stacked cavities. While the illustrated embodiments generally show stacked cavities where at least the material supply ports are aligned, in various non-limiting embodiments, cavities may be stacked such that one or more cavities are not aligned, e.g., cavities may be staggered or offset at uniform or non-uniform intervals.

It is to be appreciated that the configuration and number of molds may generally be related to the size and number of pieces to be cast and the volume of the sprue. For example, in various non-limiting embodiments, casting apparatuses may comprise a plurality of molds positioned about a rotation axis. The plurality of molds may each define a vertical stack of a plurality of cavities. Each of the plurality of cavities may define a plurality of linearly arranged cast pieces. Thus, depending on the configuration, various embodiments of the casting apparatuses may produce two to many hundreds of castings in a single casting run. That is, casting apparatuses comprising, for example, two to ten molds, each mold defining two to ten cavities, and each cavity defining two to six cast pieces, may produce between 8 and 600 cast pieces.

In the present description, other than in the operating examples or where otherwise indicated, all numbers expressing quantities or characteristics of elements, ingredients and products, processing conditions, and the like are to be understood as being modified in all instances by the term "about." Accordingly, unless indicated to the contrary, any numerical parameters set forth in the following description are approximations that may vary depending upon the desired properties one seeks to obtain in the apparatuses and methods according to the present disclosure. At the very least, and not as an attempt to limit the application of the doctrine of equivalents to the scope of the claims, each numerical parameter should at least be construed in light of the number of reported significant digits and by applying ordinary rounding techniques.

This disclosure describes various elements, features, aspects, and advantages of various non-limiting embodiments of centrifugal casting apparatuses and methods thereof. It is to be understood that certain descriptions of the various non-limiting embodiments have been simplified to illustrate only those elements, features and aspects that are relevant to a more clear understanding of the disclosed embodiments, while eliminating, for purposes of brevity or clarity, other elements, features and aspects. It is appreciated that certain features, which are, for clarity, described in the context of separate embodiments, may also be provided in combination in a single embodiment. Conversely, various features of the invention, which are, for brevity, described in the context of a single embodiment, may also be provided separately, in any suitable subcombination, or as suitable in any other described embodiment. For example, while the cavities are generally shown to extend along a horizontal operating plane, in various non-limiting embodiments, cavities may extend at positive and/or negative angles with respect to a horizontal operating plane. Additionally, certain features described in the context of various embodiments are

24

not to be considered essential features of those embodiments, unless the embodiment is inoperative without those elements.

Although the foregoing description has necessarily presented only a limited number of embodiments, those of ordinary skill in the relevant art will appreciate that various changes in the apparatuses and methods and other details of the examples that have been described and illustrated herein may be made by those skilled in the art, and all such modifications will remain within the principle and scope of the present disclosure as expressed herein and in the appended claims. Those having ordinary skill, upon reading the present description, will readily identify additional centrifugal casting apparatuses and methods and may design, build, and use additional centrifugal casting apparatuses and methods along the lines and within the spirit of the necessarily limited number of embodiments discussed herein. It is understood, therefore, that the present invention is not limited to the particular embodiments or methods disclosed or incorporated herein, but is intended to cover modifications that are within the principle and scope of the invention, as defined by the claims. It will also be appreciated by those skilled in the art that changes could be made to the non-limiting embodiments and methods discussed herein without departing from the broad inventive concept thereof.

What is claimed is:

1. A mold structured for operative association with a rotatable assembly of a centrifugal casting apparatus, the mold comprising:

at least one cavity having an entry port structured to receive molten material in a general direction of centrifugal force generated by rotation of the rotatable assembly; and,

a gate in communication with the entry port of the at least one cavity, wherein the gate includes at least one tapered portion positioned adjacent to the entry port of the at least one cavity, wherein an average cross-sectional area defined by the at least one tapered portion of the gate is greater than a cross-sectional area defined by the entry port of the at least one cavity.

2. The mold of claim 1, wherein the at least one tapered portion includes multiple tapered sub-portions.

3. The mold of claim 1, wherein the tapered portion extends around substantially the entire cross-sectional area of a portion of the gate adjacent to the entry port of the at least one cavity.

4. The mold of claim 1, wherein the at least one tapered portion extends a longitudinal distance from the entry port of the at least one cavity.

5. The mold of claim 4, wherein the longitudinal distance extends from the entry port of the at least one cavity to a sprue chamber of the rotatable assembly.

6. The mold of claim 1, wherein the at least one tapered portion extends around less than the entire cross-sectional area of a portion of the gate adjacent to the entry port of the at least one cavity.

7. The mold of claim 1, wherein the at least one tapered portion defines a taper angle in the range of greater than zero degrees to 90 degrees.

8. The mold of claim 1, wherein the average cross-sectional area defined by the at least one tapered portion of the gate is in the range of greater than 100% to 150% of the cross-sectional area defined by the entry port of the at least one cavity.

9. The mold of claim 1, wherein the at least one cavity includes the at least one tapered portion.

## 25

**10.** A casting mold structured for operative association with a rotatable assembly of a centrifugal casting apparatus, the casting mold comprising:

at least one cavity having an entry port structured to receive molten material in a general direction of centrifugal force generated by rotation of the rotatable assembly; and,

a gate in communication with the entry port of the at least one cavity, wherein the gate includes at least one tapered portion positioned adjacent to the entry port of the at least one cavity;

wherein the casting mold is a reusable casting mold; wherein an average cross-sectional area defined by the at least one tapered portion of the gate is greater than a cross-sectional area defined by the entry port of the at least one cavity.

**11.** The casting mold of claim **10**, wherein the casting mold comprises at least one of iron, an iron alloy, steel, and graphite.

**12.** The casting mold of claim **10**, wherein the casting mold is a reusable steel mold.

**13.** The casting mold of claim **10**, wherein a volume of a length of the gate is greater than a volume of an equivalent length of the at least one cavity.

## 26

**14.** The casting mold of claim **10**, wherein the at least one tapered portion includes multiple tapered sub-portions.

**15.** The casting mold of claim **10**, wherein the tapered portion extends around substantially the entire cross-sectional area of a portion of the gate adjacent to the entry port of the at least one cavity.

**16.** The casting mold of claim **10**, wherein the at least one tapered portion extends a longitudinal distance from the entry port of the at least one cavity.

**17.** The casting mold of claim **16**, wherein the longitudinal distance extends from the entry port of the at least one cavity to a sprue chamber of the rotatable assembly.

**18.** The casting mold of claim **10**, wherein the at least one tapered portion extends around less than the entire cross-sectional area of a portion of the gate adjacent to the entry port of the at least one cavity.

**19.** The casting mold of claim **10**, wherein the at least one tapered portion defines a taper angle in the range of greater than zero degrees to 90 degrees.

**20.** The casting mold of claim **19**, wherein the average cross-sectional area defined by the at least one tapered portion of the gate is in the range of greater than 100% to 150% of the cross-sectional area defined by the entry port of the at least one cavity.

\* \* \* \* \*